

## UNITED STATES PATENT OFFICE

2,352,669

## LUBRICATING OIL COMPOSITION

Paul R. Van Ess, Berkeley, and Ellis R. White,  
Albany, Calif., assignors to Shell Development  
Company, San Francisco, Calif., a corporation  
of Delaware

No Drawing. Application December 26, 1941,  
Serial No. 424,544

9 Claims. (Cl. 252—33)

This application is a continuation-in-part of our application Serial No. 376,330, filed January 28, 1941.

This invention relates to compounded lubricating oils containing added ingredients which improve their properties in one or more important respects. It also deals with the addition of oil-soluble addition agents to compounded mineral oils to produce lubricating oils of improved anti-wear properties for internal combustion engines. More particularly, it deals with the addition to lubricating oils of certain oil-soluble allophanates, which compounds have the property of modifying or reducing the hardness of carbon formed on pistons, and of preventing the baking of carbon in piston grooves to the point of hardness and thus preventing the sticking of piston rings when running internal combustion engines for long periods of time.

It is known that in modern internal combustion engines such as aviation gasoline engines, due to their high power output and their relatively high operating temperatures, or high speed Diesel engines due to incomplete combustion of the fuel, piston rings have a tendency to become stuck in the grooves and the pistons tend to become worn.

The carbon deposited in internal combustion engines may be considered of two kinds, depending on the type of oil used. High-viscosity index mineral oil tends to form hard carbon which may cause severe scratching of parts of the piston, particularly top lands as well as piston rings, etc.; while low-viscosity index oils in general form a softer carbon which does not scratch or scuff so badly. The presence of detergents in lubricating oils usually increases the tendency to scratch. Thus it is known that lubricating oils containing about 25% to 5% of oil-soluble detergents, such as the salts of polyvalent metals, or of organic amines, with detergent-forming acids, may cause damage to the top lands of pistons due to scuffing. Detergent-forming acids are, for example, naphthenic, aromatic carboxylic, hydroxy aromatic carboxylic, paraffin carboxylic; amino, hydroxy, chlorine or sulfur substituted paraffin carboxylic; rosin, petroleum sulfonic, alkyl aromatic sulfonic, phosphoric or phosphite ester, etc., acids. Other detergents having similar effects are, for instance, voltolized fatty or mineral oils, voltolized paraffin wax, polymers obtained by polymerization of unsaturated oils with  $BF_3$ , etc.

We have discovered that certain allophanates and thio-allophanates are capable of modifying

and softening hard carbon, so that well-refined lubricating oils containing oil-soluble detergents which heretofore caused too much scuffing can be used successfully, by adding small amounts of these allophanates. Oils so compounded have the valuable combination of properties of keeping the piston clean, retarding or preventing ringsticking, positively reducing wear, and overcoming and preventing piston scuffing and scratching. If desired, oxidation inhibitors, corrosion inhibitors, extreme pressure compounds, etc., may be added further to improve the desirable properties of the compounded oils containing the above combination of addition agents.

In stating that the allophanates modify the carbon formation on the piston, we mean that instead of the usual hard, tough, adhesive deposits, we find that the carbon formed in the presence of the allophanates is a soft, velvety, non-adherent deposit which is almost oily in character. Such deposits are so non-adherent they may be removed by wiping with the finger or a soft cloth, leaving a clean metal surface. No explanation can be offered for the above-observed phenomenon.

According to this invention, allophanates which are added to lubricating oils containing a sufficient amount of a detergent normally to cause scratching or scuffing of the pistons, for example, in Caterpillar Diesel engines, possess the following formula:



In this formula  $X$  represents oxygen or sulfur;  $R_2$  and  $R_3$  are hydrogen or hydrocarbon radicals, preferably hydrogen;  $R_1$  is a saturated alicyclic radical having at least 12 carbon atoms.

The hydrocarbon radicals  $R_2$  and  $R_3$  may contain preferably not more than one polar neutral or basic substituent. Suitable substituents are, for example, halogen,  $-CN$ ,  $-OH$ ,  $-OR$ ,  $-COR'$ ,  $-COOR'$ ,  $-NH_2$ ,  $-NHR'$ ,  $-NR'R''$ ,  $-SR'$ , wherein  $R'$  and  $R''$  are hydrocarbon radicals such as alkyl, aryl, aralkyl, and cycloalkyl radicals.

To be active in the matter of softening carbon deposits, it is normally necessary that the allophanates be soluble in the oil to be improved.

Normally the alicyclic radical  $R_1$  is sufficient to insure the necessary oil-solubility.

Preferred  $R_1$  radicals are those having at least two aliphatic rings, which may be condensed, and each portion having at least one branched alkyl radical. Such bi-alicyclic radicals may be obtained, for example, by hydrogenation of suitable naphthalene derivatives, as for example, a secondary or tertiary alkyl naphthol to produce the corresponding alkyl decalols; or by suitably condensing aliphatic ketones to produce unsaturated bicyclic ketones which may then be hydrogenated to the corresponding alcohols, closely resembling the above decalols.

The amounts of our allophanates to be added to the hydrocarbon oils will vary with the type of improvement to be achieved and with the severity of the hard carbon normally formed by the oil. In general, the amounts required vary from 1% to 10%, and preferably from .5% to 5%.

One group of detergents which is extremely effective in preventing ringsticking is known to comprise the salts of polyvalent metals with organic sulfonic acids, preferably the so-called oil-soluble petroleum sulfonic acids, also known as mahogany acids. Polyvalent metals suitable for this purpose are, particularly, Mg, Ca, Sr, Ba, Zn, Cd, Al, Sn, Pb, Bi, Cr, Mn, Co, Ni. However, these sulfonate detergents unfortunately cause unusually severe scuffing and scratching of the pistons. We have found that our allophanates are, therefore, particularly useful in combination with these sulfonates in that this combination takes full advantage of the highly desirable detergent property of the sulfonate without allowing the disadvantages to make themselves felt.

The presence of oxidation inhibitors in addition to detergents and allophanates is desirable not only to protect these addition agents as well as the oil from rapid destruction by oxidation, but also to prevent corrosion which may be caused by the detergent.

For our purposes, the oxidation inhibitors may roughly be divided into two groups: the phenolic type and the aryl amine type. Of these two, we have found that the latter are in general more useful. Especially valuable are those amines which contain at least one aromatic nucleus having two or more condensed aromatic rings. Thus, preferred anti-oxidants are, for example, the naphthylamines: primary, secondary, or tertiary alkyl, aryl, or aralkyl radicals, are attached to an aromatic nucleus or preferably to the nitrogen atom, or both, such as phenyl alpha or beta naphthylamine, tetraline naphthylamine, alpha alpha, alpha beta, or beta beta di-naphthylamines, various phenanthryl, anthryl, or picyl naphthylamines, xenyl naphthylamines, benzyl phenyl naphthylamines, di-phenyl naphthylamines, phenyl xenyl naphthylamines, di-xenyl naphthylamines; also, various phenanthryl, anthryl, or picyl phenyl amines, etc.

If desired, however, other oxidation inhibitors may be used as well, such as alkyl phenyl amines, di-phenyl amines; or alkyl phenols, preferably containing at least two alkyl radicals in 2, 4, or 6 positions to the OH radical, at least two alkyl radicals being linked to the aromatic nucleus through a tertiary carbon atom; or alpha or beta naphthols, alkylated naphthols, phenols, or naphthols containing ether, thio ether, etc., linkages, polyhydric alkyl benzenes or naphthalenes, such as alkylated catechol, etc. Suitable amounts of oxidation inhibitors usually vary between about .01% to 1%.

Other types of inhibitors may be added, such as corrosion inhibitors, which are not anti-oxidants, or extreme pressure compounds which may contain radicals comprising elements of the group consisting of S, P, or Cl, provided these elements are attached in such a manner that they do not readily liberate corrosive compounds such as free sulfur, chlorine, or phosphoric acid, under conditions of lubrication to which crankcase oils are usually exposed. Also, mixtures of different inhibitors are often very useful.

In accordance with the known fact that high-viscosity index oils cause more scuffing of pistons than low-viscosity oils, the combination of detergents and allophanates is particularly useful in oils of relatively high viscosity, e. g., oils having 50 viscosity index or higher.

The following examples further illustrate the invention:

#### Example I

An S. A. E. 30 lubricating oil having a viscosity index of 55, containing 2.25% of calcium petroleum sulfonate (produced by converting a commercial mahogany soap to the calcium salt), 25 0.25% phenyl alpha naphthylamine and 1.0% of an allophanate of a  $C_{18}$  saturated bicyclic alcohol (produced by the condensation of acetone and hydrogenation) was subjected to a 126-hour test in a Caterpillar test engine operated at 850 R. P. M. and at 16.7 B. H. P. At the end of the run, the piston rings were free, the piston was clean, and the top land was free of hard carbon; the metal was not scuffed. The amount of carbon deposit at the bottom of the top ring groove 35 was small.

#### Example II

An S. A. E. 30 lubricating oil containing 9% of rapeseed mild voltol as a detergent, 0.1% n-butyl arsine disulfide as a corrosion inhibitor and 0.75% of  $C_{18}$  saturated cyclo-alkyl allophanate as carbon modifier was subjected to a 36-hour test in a Chevrolet test engine under severe operating conditions (3150 R. P. M.). At the end of the 40 test the engine parts were free from lacquer and carbon deposits.

We claim as our invention:

1. An improved lubricant comprising a mineral lubricating oil having dissolved therein a small amount each of an oil-soluble detergent normally tending to promote scratching or scuffing of pistons and an oil-soluble allophanate selected from the group consisting of allophanates of alicarbocyclic alcohols and thio-alcohols, having at least 55 12 carbon atoms.
2. An improved lubricant comprising a mineral lubricating oil having dissolved therein a relatively small amount each of an oil-soluble detergent normally tending to promote scratching or scuffing of pistons, an amine anti-oxidant, and an oil-soluble allophanate selected from the group consisting of allophanates of alicarbocyclic alcohols and thio-alcohols, having at least 60 12 carbon atoms.
3. An improved lubricant comprising a mineral lubricating oil having dissolved therein .25% to 5% of an oil-soluble detergent normally tending to promote scratching or scuffing of pistons and .1% to 10% of an oil-soluble allophanate selected from the group consisting of allophanates of alicarbocyclic alcohols and thio-alcohols, having at least 65 12 carbon atoms.
4. An improved lubricant comprising a mineral lubricating oil having dissolved therein .25% to 70 5% of an oil-soluble detergent normally tending

to promote scratching or scuffing of pistons and from .5% to 5% of an oil-soluble allophanate selected from the group consisting of allophanates of alicarbocyclic alcohols and thio-alcohols, having at least 12 carbon atoms.

5. An improved lubricant comprising a mineral lubricating oil having dissolved therein .25% to 5% of an oil-soluble detergent normally tending to promote scratching or scuffing of pistons, .1% to 1% of an amine anti-oxidant, and .1% to 10% of an oil-soluble allophanate selected from the group consisting of allophanates of alicarbocyclic alcohols and thio-alcohols, having at least 12 carbon atoms.

6. An improved lubricant comprising a mineral lubricating oil having dissolved therein .25% to 5% of a polyvalent metal salt of petroleum

sulfonate, and .1% to 10% of an oil-soluble allophanate selected from the group consisting of allophanates of alicarbocyclic alcohols and thio-alcohols having at least 12 carbon atoms.

5 7. An improved lubricant comprising a mineral lubricating oil having dissolved therein .25% to 5% calcium petroleum sulfonate, .1% to 1% phenyl alpha naphthylamine, and .1% to 10% of a branched-chain alkyl decalol allophanate.

8. The composition of claim 7 wherein said decalol has 18 carbon atoms.

9. The composition of claim 7 in which the viscosity index of the mineral lubricating oil is above 50.

PAUL R. VAN ESS.  
ELLIS R. WHITE.